

## UNITED STATES PATENT OFFICE

2,114,629

## COMPOSITE BEARING METAL

William E. McCullough, Detroit, Mich., assignor  
to Bohn Aluminum & Brass Corporation, De-  
troit, Mich., a corporation of Michigan

No Drawing. Application July 12, 1937,  
Serial No. 153,201

4 Claims. (Cl. 75—163)

The invention relates to metal compositions of the general type known as copper lead alloys and which are extensively used in the forming of bearings for working parts. It is the object of the invention to obtain a composition of this type having physical characteristics which better adapt it for use in bearings, particularly those designed for heavy duty and high speeds.

It has now been well demonstrated that the fatigue endurance (resistance to cracking) of the leaded bronze lining of steel-backed bearings is greater with certain types of metal structure than with others. For instance, when ordinary copper is melted and commercial lead is added to the molten copper, it is difficult to retain more than 30% of lead in the cast lining at a point  $\frac{1}{2}$  of an inch removed from the steel back, and the copper invariably assumes a definite dendritic form, with lead filling in the spaces between the branches of the copper dendrites.

When such bearings are run in an engine they are subjected to stresses which result in a cracking of the lining and eventually the destruction of the bearing through the cracked pieces loosening from the shell. This is characteristic of the failure of the majority of aircraft engine bearings, the cracked areas usually occurring at the points of greatest stress. I have discovered that one cause of such failures is the dendritic structure of the copper content, which while holding the lead between dendrites does not sufficiently integrate or hold together all parts of the structure. I have further discovered an improved composition and method of forming the same, in which the copper forms a substantially continuous matrix completely enclosing each lead globule. Such composition has greatly improved physical characteristics, particularly in that it lessens the danger of cracking and at the same time improves the lubricating or bearing quality of the metal.

My improved composition is formed by the addition to the copper and lead of a metallic element which has a strong modifying action and prevents a dendritic formation of the copper content. Various metals may be used for this purpose, but not all are desirable because of the other properties of a more or less detrimental character. For instance, a small amount of tin added to the composition will have the desired result in changing the structure of the copper content, but it is, nevertheless, detrimental in that it decreases the lubricating characteristic of the lead with greater danger of seizure. I have discovered that a small quantity of metallic mag-

nesium added to the composition will have the beneficial effect and will avoid the detrimental effect of the tin.

My improved composition may be manufactured by various methods. In one method producing satisfactory results a small but definite percentage of magnesium is first alloyed with the molten lead which is then cast into ingots. The percentage of magnesium may vary from 0.05% to 5%, this magnesium being readily soluble in the molten lead, and requiring no special precautions during melting. The lead-magnesium alloy is then cast into ingot or other suitable forms. Copper is then melted, preferably, but not necessarily, in a crucible type of furnace, which may be heated in any conventional way. Commercial pig lead may then be added to the molten copper to a desired amount, but I prefer to add approximately 40% of such ordinary pig lead. A further addition of magnesium bearing lead is then made to the molten mixture, sufficient to add a small percentage of magnesium to the molten metal. My experiments have shown that this amount of magnesium may be varied from .005% by weight to 1% by weight, following which the metal is cast into a previously heated steel shell in any conventional way.

I have also found that metallic magnesium may be added directly to the molten copper-lead mixture with apparently the same result, but I find it more convenient to control the exact amount of magnesium so added through previously alloying it with lead, as described. In my experiments fifty consecutive heats of metal have been melted and cast, using magnesium additions over the range previously set forth, with not in a single instance producing a leaded bronze lining having a dendritic structure, the lining being invariably of the matrix type.

My experiments have also shown that the addition of magnesium may be made through the compression into small tablets of a mixture of 90% copper powder and 10% magnesium powder, these tablets being added to a molten mixture of copper and lead just before casting. The cast metal after this treatment with the copper-magnesium composition shows the same non-dendritic character as when the magnesium-lead alloy is used. Various proportions of copper and magnesium may, of course, be employed for this purpose. It is less convenient, however, to use the magnesium in powdered form than in the form of lead-magnesium alloy. I have also added an alloy of  $\frac{1}{2}\%$  magnesium in copper with similar results.

While I have described the treatment of the molten copper-lead metal with metallic magnesium, with copper-magnesium compressed from powdered metals, with copper-magnesium alloy, and the treatment with a lead-magnesium alloy, it is obvious that there would be various other methods of treating the metal with magnesium, for instance, with magnesium vapor, etc., but I consider all such other possible methods of 5 treating a molten mixture of copper and lead with magnesium in any form prior to casting in final form would fall within the scope of my discovery.

The magnesium additions have covered a range 10 over the various samples and have shown a residual magnesium in the bearing lining varying from a spectrographic trace up to a chemical content of 0.42% of metallic magnesium, with no basic difference in structural type of the lining although it appears that the addition of magnesium in the smaller amounts results in a somewhat finer distribution of the lead throughout the copper matrix. A further benefit from the addition of magnesium has been that the 15 copper retains more lead in the matrix than when tin is used or when no addition agent is used and bearings have been cast with 40% of lead evenly dispersed throughout the matrix at a distance of  $\frac{3}{2}$  of an inch from the steel shell.

that being the thickness of lining usually employed in such bearings in the finished state.

What I claim as my invention is:

1. A bearing composed of copper, lead, and magnesium in the proportions of not less than 55 per cent by weight of copper nor more than 5 45 nor less than 20 per cent by weight of lead and from a spectrographic trace to 5.0 per cent by weight of magnesium.

2. A composition of matter composed of from 55 to 80 per cent by weight of copper, from 20 to 10 45 per cent by weight of lead and from a spectrographic trace to 1.0 per cent by weight of magnesium.

3. A bearing lining for steel-backed internal 15 combustion engine bearings composed of from 55 to 80 per cent by weight of copper, from 20 to 45 per cent by weight of lead and having been treated with 0.005 per cent to 1.0 per cent by weight of magnesium, said bearing lining being 20 characterized by a non-dendritic type of micro-structure.

4. A composition of matter composed of copper, lead and magnesium in the proportions of lead not more than 45% nor less than 20% by 25 weight, magnesium from a spectrographic trace to 5.0% by weight and the balance of copper.

WILLIAM E. McCULLOUGH.